# EUROPEAN PATENT SPECIFICATION

(11) **EP 2 978 867 B1**
(45) Date of publication and mention of the grant of the patent: **19.04.2017**
(21) Application number: 14720688.2
(22) Date of filing: 20.03.2014
(51) Int. Cl.: C22C 5/06

(54) **ALLOY FOR THE PRODUCTION OF JEWELS**
LEGIERUNG FÜR DIE HERSTELLUNG VON JUWELEN
ALLIAGE POUR LA PRODUCTION DE BIJOUX

(30) Priority: 26.03.2013 IT VI20130084
(43) Date of publication of application: 03.02.2016
(73) Proprietor: 1KTG SRL, 36057 Arcugnano (VI) (IT)
(72) Inventor: GARFARINO, Mario, 36057 Arcugnano (IT)
(74) Representative: Bonini, Ercole
(86) International application number: PCT/IB2014/000408
(87) International publication number: WO 2014/155178

(56) References cited:
- US-A- 4 396 578
- US-A1- 2008 095 659

## Description

### Technical field of the invention

The invention concerns an alloy for the production of jewels, in particular trinkets. The invention concerns also objects, in particular jewels and trinkets produced with this alloy, as well as the use of the alloy for the production of jewels.

### State of the art

In the market of jewellery and costume jewellery a large number of gold alloys or alloys of other precious metals, like for example platinum, are known and used to make jewels.

Gold and platinum are metals that do not oxidize easily but they are very expensive. The weight of gold and platinum is relatively high, which limits the size that can be reasonably obtained for the jewels, in particular in the case of earrings. In order to be able to offer jewels also at reasonable prices, the market of costume jewellery has developed several alloys with a low gold and platinum content that are less expensive than gold alloys but pose several drawbacks. In order to prevent the oxidation of the alloy and therefore the alteration of its appearance, similar to that of precious alloys, it is necessary to coat the item, for example by means of a plating process carried out using galvanising methods. This layer, however, is subject to wear. Due to the oxidation processes, in most cases the alloys that replace the traditional gold alloys do not maintain their gilded/platinum plated appearance over time and need to be frequently cleaned. Moreover, often these alloys do not imitate the precious metal and its alloys perfectly in terms of external appearance, that is, in terms of colour and degree of brightness. In particular, the market offers only a few alloys with a low content of precious metals that look like white gold. Document US 2008/095659 A1 describes an alloy composition that is intended for use as alternative to the more expensive white gold.

### Presentation of the invention

The object of the present invention is to propose an improved alloy that overcomes the drawbacks listed above. The object of the present invention is mainly to propose an alloy with a low precious metal carat rating that, in addition to not oxidizing easily and having good workability for the needs of the jewellery sector, imitates the aspect and the brightness of white gold.

The objects mentioned above and others that are highlighted in greater detail below are achieved by an alloy for the production of jewels that is constituted by: 4 - 10%, preferably 5 - 10%, more preferably 6 - 10% zinc by weight; 0.1 - 4.3% gold by weight; 8 - 20% copper by weight; 1 - 6% indium by weight; 0 - 4.3% platinum by weight; 0 - 4.3% palladium by weight; 0 - 10%, preferably 0 - 1.5% by weight of a combination of nickel and rhodium preferably with a weight ratio of 1:1; 0 - 0.5% by weight of one or more auxiliary elements, selected among iridium, germanium, silicon, osmium, tin and gallium, wherein the rest is constituted by silver.

It is to be understood that the alloys described herein can always contain other elements, meaning elements that are not listed as components that make up the alloy, in the form of traces in overall quantities up to 0.2% by weight, preferably up to 0.1% by weight. These traces derive from impurities present in the raw materials or are residues of auxiliary materials used during the production or processing of the alloy.

In order to affect the fluidity of the molten material and the suitability of the material for precision casting, forming (in this case silicon-free alloys are preferably used) or welding, and to obtain a finer grain, the expert in the art, thanks to his/her general knowledge of the matter, changes the percentages of the auxiliary components.

The alloy according to the invention is advantageously in the colour of white gold. The variation in the content of metals or combinations of metals that are yellow/red compared to metals with a silvery colouring makes it possible to obtain different hues within the colour that in the sector of jewellery is considered as white gold colour.

Advantageously, in the alloys according to the invention that contain nickel there is rhodium in a weight ratio of 1:1 with respect to nickel, in order to bind nickel and prevent it from detaching from the alloy and therefore to reduce the allergenic nature of the alloy itself.

Even with a low carat rating of gold, platinum and palladium, respectively, it has been possible to produce alloys that do not oxidize easily and imitate the colour of white gold while at the same time showing a high degree of brightness.

Moreover, the alloy is very sturdy, elastic, easy to clean, polish and machine and has good lapping values, partly better than those of other alloys with higher carat rating.

According to an advantageous embodiment of the invention, the alloy does not contain iridium, germanium, silicon, osmium, tin and gallium as elements that make up the alloy. As explained above, the alloy, in any case, can contain these elements within the group consisting of traces of other elements.

The variant embodiments described below are the compositions that in the search for economic alloys with low precious metal carat rating have proved to be particularly suited to be used to make trinkets, because they do not oxidize easily, are easy to machine and shiny, and imitate the shades of the alloys known as white gold.

A preferred variant embodiment of the invention concerns an alloy whose silver content corresponds to 55 - 75% by weight. Obviously, the sum of the weights of the components of the alloy as indicated above makes up a total of 100% by weight.

Advantageously, the alloy according to the invention comprises 8 - 15% copper by weight, preferably 14 - 15% copper by weight. Contrary to expectations, this percentage represents a good compromise between a reduction of yellow in the alloy and a satisfactory structure in terms of sturdiness and workability of the alloy.

In a preferred variant embodiment of the invention, the content of indium in the alloy according to the invention corresponds to 1 - 2% by weight. Even relatively small quantities of indium produce a considerable whitening effect.

Advantageously, the alloy according to the invention comprises approximately 4.17% gold by weight. In preferred variant embodiments of the invention, the alloy also comprises approximately 4.17% platinum or palladium by weight or approximately 4.17% platinum by weight and approximately 4.17% palladium by weight.

According to another variant embodiment, the alloy according to the invention comprises 4.17% by weight of one or more precious metals selected among gold, palladium and platinum.

According to a further variant embodiment, the alloy according to the invention comprises 8.34% by weight or 12.51% by weight of one or more precious metals selected among gold, palladium and platinum, wherein gold is preferably present in concentrations of 4.17% by weight. These alloys correspond to alloys with low precious metal carat ratings: for example, 1 carat gold and alternatively 1 carat gold plus 1 or 2 carats platinum and/or palladium. Even with maximum 3 carats of precious metals (gold, platinum and palladium) it has been possible to obtain an alloy that does not oxidize easily, is sufficiently hard and elastic, suited to be worked with the techniques in use in the jewellery sector, very bright and in the colour of white gold.

In order for the hardness of the alloy to be increased, the same comprises 1 - 1.5% nickel by weight and, due to the reasons explained above, also 1 - 1.5% rhodium by weight.

A much preferred alloy according to the invention is constituted by 19 - 20% copper by weight, 4 - 5% zinc by weight, approximately 4.17% gold by weight, 1 - 2%, preferably approximately 2% indium by weight, and the remaining percentage needed to reach 100% by weight is silver. The alloy is characterized by optimal workability for the jewellery sector, considerable brightness and a white gold colour thanks to which it can be mistaken for real white gold.

The invention furthermore concerns the use of the alloy according to the invention for the production of jewels, in particular trinkets.

A third aspect of the invention concerns an item, preferably a jewel or a trinket, produced with an alloy according to the invention.

Other possible items that can be produced with an alloy according to the invention are, for example, coins, tableware, candle holders or other items of art handicraft.

It should be understood that the indicated values (their percentages by weight) always include also values that can be considered equivalent from the point of view of weighing accuracy and analysis of the individual components.

The alloy according to the invention is suited to be used in the processing cycles that are typical of the jewellery sector.

The invention achieves the object to provide an economic alloy with low carat rating of gold, platinum and palladium that, in addition to not oxidizing easily and having good workability, imitates the appearance of white gold and is considerably bright.

Further variant embodiments of the invention are described in the dependent claims.

In the production stage, the alloy, its use and the items manufactured with this alloy that is the subject of the invention can be subjected to further modifications or construction variants that are not described herein. Said modifications or variants must all be considered protected by the present patent, provided that they fall within the scope of the claims expressed below.

### Description of preferred embodiments of the invention

The production of the alloy follows the methods known in the art and the general knowledge of the expert in the art for producing alloys containing gold, silver, brass, etc. The components of the alloy can be combined together starting from the pure metals and/or corresponding alloys, like for example brass, for example brass containing 70% copper by weight and 30% zinc by weight. These methods are not described herein for the sake of brevity.

The following table 1 lists some examples of embodiment of alloys according to the invention:

**Table 1**

| copper [w%] | zinc [w%] | indium [w%] | palladium [w%] | platinum [w%] | gold [w%] | nickel and rhodium [w%] | silver [w%] | other [w%] |
|---|---|---|---|---|---|---|---|---|
| 8-15 | 5-10 | 1 -2 | 0 - 4.3 | 0 - 4.3 | 0.1 - 4.3 | 0 | balance to reach 100% by weight | 0-0.5 |
| 8-15 | 5-10 | 1-2 | 0 | 0 | 4.17 | 0 | balance to reach 100% by weight | 0-0.5 |
| | | | 4.17 (alone or in combination with other metals) | | 4.17 | | | |
| | | | 4.17 | 4.17 | 4.17 | | | |
| 14-15 | 5-10 | 1-2 | 0 - 4.3 | 0 - 4.3 | 0.1 - 4.3 | 0 | balance to reach 100% by weight | 0-0.5 |
| 19-20 | 4-5 | 2 | 0 | 0 | 4.17 | 0 | balance to reach 100% by weight | 0-0.5 |

The abbreviation "w%", known in the sector, means "% by weight". Possible traces of other elements that can be contained in the alloy up to an overall maximum of 0.2% by weight, preferably in concentrations ≤ 0.1% by weight, have not been indicated.

## Claims

1. Alloy for the production of jewels, constituted by: 4 - 10%, preferably 5 - 10%, more preferably 6 - 10% zinc by weight; 0.1 - 4.3% gold by weight; 8 - 20% copper by weight; 1 - 6% indium by weight; 0 - 4.3% platinum by weight; 0 - 4.3% palladium by weight; 0 - 10%, preferably 0 - 1.5% by weight of a combination of nickel and rhodium preferably with a weight ratio of 1:1; 0 - 0.5% by weight of one or more auxiliary elements selected among iridium, germanium, silicon, osmium, tin and gallium, wherein the rest is constituted by silver.

2. Alloy according to claim 1, **characterized in that** its silver content corresponds to 55 - 75% by weight.

3. Alloy according to claim 1 or 2, **characterized in that** its copper content corresponds to 8 - 15% by weight, preferably 14 - 15% by weight.

4. Alloy according to claim 2 or 3, **characterized in that** its indium content corresponds to 1 - 2% by weight.

5. Alloy according to any of the preceding claims, **characterized in that** it comprises 4.17% gold by weight.

6. Alloy according to claim 5, **characterized in that** it furthermore comprises 4.17% platinum and/or palladium by weight, or 4.17% platinum by weight and 4.17% palladium by weight.

7. Alloy according to any of the preceding claims, **characterized in that** it comprises 1 - 1.5% nickel by weight and 1 - 1.5% rhodium by weight.

8. Alloy according to claim 1 or 2, **characterized in that** it is constituted by 19 - 20% copper by weight, 4 - 5% zinc by weight, 4.17% gold by weight, 1 - 2%, preferably 2% indium by weight, while the remaining percentage needed to reach 100% by weight is silver.

9. Use of the alloy according to any of the preceding claims for the production of jewels, in particular trinkets.

10. Item, preferably a jewel or a trinket, produced from an alloy according to any of the claims from 1 to 8.

## Patentansprüche

1. Legierung für die Herstellung von Schmuckstücken, Folgendes umfassend: 4 - 10%, vorzugsweise 5 - 10%, besonders bevorzugt 6 - 10% Gewichtsanteil Zink; 0,1 - 4,3% Gewichtsanteil Gold; 8 - 20% Gewichtsanteil Kupfer; 1 - 6% Gewichtsanteil Indium; 0 - 4,3% Gewichtsanteil Platin; 0 - 4,3% Gewichtsanteil Palladium; 0 - 10%, vorzugsweise 0 - 1,5% Gewichtsanteil einer Kombination aus Nickel und Rhodium, vorzugsweise mit einem Gewichtsverhältnis von 1:1; 0 - 0,5% Gewichtsanteil eines oder mehrerer Zusatzelemente, ausgewählt unter Iridium, Germanium, Silizium, Osmium, Zinn und Gallium, wobei der Rest aus Silber besteht.

2. Legierung gemäß Patentanspruch 1, **dadurch gekennzeichnet, dass** der Silbergehalt 55 - 75% Gewichtsanteil entspricht.

3. Legierung gemäß Patentanspruch 1 oder 2, **dadurch gekennzeichnet, dass** ihr Kupfergehalt 8 - 15% Gewichtsanteil und vorzugsweise 14 - 15% Gewichtsanteil entspricht.

4. Legierung gemäß Patentanspruch 2 oder 3, **dadurch gekennzeichnet, dass** ihr Iridiumgehalt 1 - 2% Gewichtsanteil entspricht.

5. Legierung gemäß eines jeden der vorstehenden Patentansprüche, **dadurch gekennzeichnet, dass** sie 4,17% Gewichtsanteil Gold enthält.

6. Legierung gemäß Patentanspruch 5, **dadurch gekennzeichnet, dass** sie des Weiteren Folgendes umfasst: 4,17% Gewichtsanteil Platin und/oder Palladium, oder 4,17% Gewichtsanteil Platin und 4,17% Gewichtsanteil Palladium.

7. Legierung gemäß eines jeden der vorstehenden Patentansprüche, **dadurch gekennzeichnet, dass** sie 1 - 1,5% Gewichtsanteil Nickel und 1 - 1,5% Gewichtsanteil Rhodium enthält.

8. Legierung gemäß Patentanspruch 1 oder 2, **dadurch gekennzeichnet, dass** sie zu 19 - 20% Gewichtsanteil aus Kupfer, zu 4 - 5% Gewichtsanteil aus Zink, zu 4,17% Gewichtsanteil aus Gold, zu 1 - 2%, vorzugsweise zu 2% Gewichtsanteil aus Indium besteht, während der verbleibende, bis zum Erreichen von 100% erforderliche Gewichtsanteil Silber ist.

9. Verwendung der Legierung gemäß eines jeden der vorstehenden Patentansprüche zur Herstellung von Schmuckstücken, insbesondere von Modeschmuck.

10. Gegenstand, vorzugsweise ein Schmuckstück oder Modeschmuck, dass aus einer Legierung gemäß eines jeden der Patentansprüche von 1 bis 8 hergestellt wird.

## Revendications

1. Alliage pour la production de bijoux, constitué de: 4 - 10% en poids, préférablement 5 - 10% en poids, plus préférablement 6 - 10% en poids de zinc; 0,1 - 4,3% en poids d'or; 8 - 20% en poids de cuivre; 1 - 6% en poids d'indium; 0 - 4,3% en poids de platine; 0 - 4,3% en poids de palladium; 0 - 10% en poids, préférablement 0 - 1,5% en poids d'une combinaison de nickel et rhodium préférablement dans le rapport de poids 1:1; 0 - 0,5% en poids d'un ou plusieurs éléments auxiliaires choisis parmi iridium, germanium, silicium, osmium, étain et gallium, où le reste est constitué d'argent.

2. Alliage selon la revendication 1, **caractérisé en ce que** le contenu en argent correspond à 55 - 75% en poids.

3. Alliage selon la revendication 1 ou 2, **caractérisé en ce que** le contenu en cuivre correspond à 8 - 15% en poids, préférablement à 14 - 15% en poids.

4. Alliage selon la revendication 2 ou 3, **caractérisé en ce que** le contenu en indium correspond à 1 - 2% en poids.

5. Alliage selon l'une quelconque des revendications précédentes, **caractérisé en ce qu'**il comprend 4,17% en poids d'or.

6. Alliage selon la revendication 5, **caractérisé en ce qu'**il comprend en outre 4,17% en poids de platine et/ou palladium, ou 4,17% en poids de platine et 4,17% en poids de palladium.

7. Alliage selon l'une quelconque des revendications précédentes, **caractérisé en ce qu'**il comprend 1 - 1,5% en poids de nickel et 1 - 1,5% en poids de rhodium.

8. Alliage selon la revendication 1 ou 2, **caractérisé en ce qu'**il est constitué de 19 - 20% en poids de cuivre, 4 - 5% en poids de zinc, 4,17% en poids d'or, 1 - 2% en poids, préférablement 2% en poids d'indium et le restant pourcentage à 100% en poids d'argent.

9. Utilisation de l'alliage selon l'une quelconque des revendications précédentes pour la production de bijoux, en particulier d'articles de fantaisie.

10. Objet, préférablement un bijou ou un article de fantaisie, réalisé à partir d'un alliage selon l'une quelconque des revendications de 1 à 8.
